

Filed Oct. 1, 1940.  
To Standard Oil Development Company, a corporation of Delaware.

## UNITED STATES PATENT OFFICE

2,373,044

## FUELS FOR COMBUSTION

Pharis Miller, Elizabeth, and Gould H. Cloud,  
Linden, N. J., assignors to Standard Oil Development Company, a corporation of Delaware

No Drawing. Application August 9, 1941,  
Serial No. 406,164

4 Claims. (Cl. 44—57)

This invention relates, in general, to improvement of hydrocarbon fuels for efficient combustion in combustion engines.

This application is a continuation-in-part of our application Serial No. 232,799, which was filed on October 1, 1938, now Patent No. 2,268,383, dated December 30, 1941. This earlier application relates to improvements in ignition qualities of fuels for high speed compression-ignition engines by additions of sulfur entirely in free form, or partly in the free form and partly combined.

The present application is concerned more specifically with the use of sulfur combined with amino groups as in hexasulfamide to improve ignition qualities of the compression-ignition engine fuels.

Combustion engines, more particularly, high speed compression-ignition engines, are generally referred to by the name of their prototype, the Diesel engine. Hydrocarbon fuels which have been found most suitable for these engines are crude oil distillates which are highly paraffinic, but these fuels are limited in supply and relatively expensive.

In consideration of increasing power and fuel economy with elimination of vibration harmful to the mechanism in the operation of compression-ignition engines, principally when the hydrocarbon fuel contains insufficient amounts of hydrocarbon compounds recognized as serving these ends by virtue of their suitable ignition qualities, the addition of various chemical substances to the fuels has been proposed.

Hydrocarbon compounds characterized by aromatic, other cyclic, and highly unsaturated hydrocarbons have poor ignition qualities as Diesel engine fuel ingredients, following from the fact that hydrocarbon fuels containing a large proportion of these compounds fail to undergo prompt and smooth combustion in representative types of engines in which unsuitable combustion is manifested by engine vibrations and annoying "knocking" sounds.

A poor ignition quality in a compression-ignition engine fuel is exhibited by an excessive ignition lag, in other words, an excessive delay between the beginning of fuel injection into the combustion chamber of the engine and the point at which ignition of the fuel sets in. In contrast, the normal paraffin hydrocarbon cetane, which serves as a standard of high ignition quality in Diesel fuel rating by recommendation of the S. A. E. Volunteer Group for Compression-Ignition Fuel Research, has a desirable minimum ignition lag. Since the ignition lag of a blend

consisting of normal cetane and the aromatic compound alpha-methyl naphthalene is shortened very nearly in proportion to the increase in percentage of cetane by volume, the ignition quality of a fuel can be measured in terms of the cetane content of such a blend. Accordingly, when the improvement in a fuel by a small amount of addition agent corresponds to an improvement by an increase of about 5% or more of cetane by volume in a blend with alpha-methyl naphthalene, such an addition agent is considered to have commercially significant effectiveness, provided the addition agent used is not very costly in comparison with the value of the fuel.

Attempts have been made to find substances effective for improving ignition qualities of Diesel fuels, but various substances determined to be effective for this purpose are not altogether satisfactory from all points of view for commercial use. For example, a number of the effective promoters, such as alkyl nitrates, are rather expensive at present, some are too unstable, some are excessively corrosive, and some are not readily dissolved in the hydrocarbon fuels.

The present invention has as its object the improvement of Diesel fuels in their ignition qualities by an agent that can be prepared inexpensively, has good stability, is readily dissolved in the hydrocarbon fuels, and is relatively less corrosive than free sulfur and a number of types of sulfur-containing substances which have been proposed as ignition promoters.

It has been found that sulfur combines with a small proportion of amino groups as in hexasulfamide which is believed to have a composition represented by the formula:



$x$  being undetermined specifically, but being usually of the order of 5 or more; and in this composition produces almost the same cetane number increase as does free sulfur when added to a Diesel fuel, while having a much lower copper strip corrosion action and higher solubility.

To obtain a combination of sulfur with the amino group, ammonia may be reacted with a sulfur chloride or sulfur may be reacted with ammonia. A convenient method used to prepare hexasulfamide in good yields is one in which ammonia is passed through a solution of sulfur monochloride in chloroform, the reaction mixture being cooled by heat exchange with a freezing mixture in the early part of the reaction to prevent violent reaction, and after darkening of color, being permitted to have an increase in tem-

perature. The admission of ammonia was continued until the reaction mixture color became salmon red. From the resulting reaction products, ammonium chloride was filtered off. Alternatively, the ammonium chloride may be removed by extraction with water. Other low boiling alkyl halide diluents, such as ethylene dichloride, may be used in place of chloroform. With increase of temperature toward the end of the reaction, the yield of hexasulfamide, forming a larger part of the reaction products, is increased while the undesired by-product, sulfur nitride, which is unstable and relatively insoluble in hydrocarbon oils, is reduced to a negligible amount.

It is possible to separate the combined sulfur and amine compound from the other reaction products so that it may be added alone to the Diesel fuel, or the sulfur reaction products, including free sulfur, may be added together to the oil. Hexasulfamide crystals may be recovered from the chloroform solution in which it is prepared by fractional crystallization due to the relatively greater solubility of the hexasulfamide in organic solvents. For example, the chloroform solution is first evaporated down to about a fourth of its original volume, then, upon addition of 95% ethyl alcohol, in excess, a by-product comprising some free sulfur comes out of solution. After filtering off the by-product precipitate, re-concentrating the filtrate, and diluting the concentrate with benzene, hexasulfamide is crystallized out from the benzene by addition of aqueous alcohol. Purified hexasulfamide, obtained by recrystallization, is insoluble in and stable towards water, odorless, non-explosive, and stable to air. Cetane number tests on a Diesel oil composed of a Colombian gas oil and containing only 1.5% of the animated sulfur show that this addition agent gives the fuel a cetane number increase of +10 or +11.

Owing to its good stability to air and moisture, and to the ease with which it is dissolved in a hydrocarbon fuel, hexasulfamide is a very suitable agent for addition to a fuel on its passage to the engine from the engine supply tank.

The proportion of hexasulfamide to be added to a hydrocarbon fuel for effecting improvement in ignition ranges from a fraction of 1% to its limit of solubility in the fuel, and, as needed. Preferably it is used in concentrations from about 0.1% to 5% by weight, although when it is used with a more potent agent, such as free sulfur, it need not be used in as large amounts to obtain a certain cetane number increase.

A gas oil boiling from about 400° F. to 700° F. or 750° F., or, in general, having a suitable boiling range and viscosity for use as a fuel in Diesel type engines, may be used as the hydrocarbon fuel. Under some circumstances, a more narrowly cut fraction, such as one distilling from 400 to 600° F. or from 500 to 700° F. may be used. Ordinarily, the hydrocarbon fuel may be said to have a boiling range above that of gasoline.

This invention makes commercially feasible the preparation of Diesel fuels giving satisfactory engine performance from crude oils, gas oils, and residual fuels having low pour points, low A. P. I.

gravities, and high heat values, such oils being procured from naphthene base, asphalt base, or mixed base stocks. Heavier and lower grades of petroleum oil, such as residual oils, are even made more suitable for slow speed engines.

The burning qualities of fractions from paraffin crudes or hydrogenated oils are also enhanced by the novel addition agent of this invention.

Small quantities of these novel addition agents 10 may be used for adapting various mixtures of hydrocarbons for use as Diesel fuels, including recycle stocks from cracking operations, non-paraffinic extracts, oils from destructive distillations of pyro-bituminous and asphaltic materials, and mixtures of these with one another or with crude petroleum fractions. With improvement in the ignition qualities of the hydrocarbon fuels mentioned by addition of inexpensive agents herein disclosed better performance of a Diesel engine operating on the improved fuel is obtained in the way of easier starting, smoother idling, silent running, and absence of shock loading.

It is not intended that this invention be limited 25 to the specific examples which are given merely for the sake of illustration, but it is desired to claim all the novelty inherent in this invention in the appended claims as broadly as the prior art permits.

Other agents for enhancing various other qualities without detracting substantially from the ignition qualities of the fuel may be admixed, such as oiliness agents, sludge dispersers, colloidal suspension dispersers and stabilizers, dyes, anti-oxidants, viscosity improvers, pour point depressants, solubilizers, gum solvents, and corrosion inhibitors. Substances such as olefins, amines, and peroxides may be mentioned as being effective for reducing any corrosive tendencies of active sulfur promoters. Also, other promoters of ignition quality may be admixed, particularly alkyl nitrates, such as amyl nitrate.

We claim:

1. A fuel for compression-ignition engines of 45 the Diesel type which comprises a hydrocarbon Diesel fuel and a sulfur-containing ignition promoter consisting essentially of hexasulfamide containing no free sulfur in an amount sufficient to improve the ignition quality of the fuel.

2. A Diesel fuel comprising a hydrocarbon Diesel fuel containing about 0.1% to about 5% by weight of hexasulfamide containing no free sulfur.

3. A method of accelerating ignition of a Diesel fuel which comprises adding to the fuel prior to its ignition a small amount of a sulfur-containing ignition promoter consisting essentially of hexasulfamide containing no free sulfur sufficient to substantially increase the cetane number value of the fuel.

4. A Diesel fuel comprising a major proportion of a hydrocarbon fuel base stock of the gas oil boiling range containing at least about 1.5% of hexasulfamide containing no free sulfur.